

S. I. CLAWSON.  
PROCESS FOR VOLATILIZING ORES.  
APPLICATION FILED AUG. 11, 1909.

1,262,453.

Patented Apr. 9, 1918.



Inventor

Selden I. Clawson  
Sturtevant & Mason  
Attorneys

Witnesses

H. Walker

C. C. Sampson

By

# UNITED STATES PATENT OFFICE.

SELDEN IRWIN CLAWSON, OF SALT LAKE CITY, UTAH.

## PROCESS FOR VOLATILIZING ORES.

1,262,453.

Specification of Letters Patent.

Patented Apr. 9, 1918.

Application filed August 11, 1909. Serial No. 512,449.

*To all whom it may concern:*

Be it known that I, SELDEN I. CLAWSON, a citizen of the United States, residing at Salt Lake City, in the county of Salt Lake, 5 State of Utah, have invented certain new and useful Improvements in Processes for Volatilizing Ores, of which the following is a description, reference being had to the accompanying drawing, and to the letters and 10 figures of reference marked thereon.

The invention relates to new and useful improvements in an apparatus and a process of volatilizing ores.

An object of the invention is to provide an 15 apparatus wherein the chlorin gas may be re-claimed from the volatile chlorids and re-used in the volatilization of the ores.

A further object of the invention is to provide a process wherein the chlorin gas 20 used in the volatilization of the ores may be re-claimed and re-used in the further volatilization action.

These and other objects will in part be 25 obvious, and will in part be hereinafter more fully disclosed.

The figure of the drawings shows more or less diagrammatically and in section an apparatus containing my improvements, and by which my improved process may be carried out.

The apparatus as herein disclosed, 30 consists of a furnace 1, which is provided with a fire box 2 and a closed chamber 3. A hopper 4 is connected by a chute 5 with a chamber 3. The gases from the fire box will encircle the closed chamber 3, heating the same to the desired temperature, and pass through 35 the pipe or stack 6. The crushed ore which may be preheated, if desired, is fed through 40 the hopper 4 and chute 5 to the chamber 3.

A pipe 7 leads through the wall of the furnace and into the chamber 3, and may be used for supplying said chamber with chlorin 45 gas to aid in the chemical action upon the ore and the carrying on of the volatilization process. The ore in the chamber 3 will practically close the chute 5, and prevent any draft through said chute.

A pipe 8 leads from the upper part of the 50 chamber 3, and conveys the gases and fumes from the chamber. A suitable door 9 may be provided, and a little air may be fed to the chamber 3 through the door, if desired; or air may be forced in with chlorin gas 5 through pipe 7.

The pipe 8 leads to a fume arrester 9,

which may be of any desired construction. As herein shown, said fume arrester is provided with side walls 10, and with a top portion 11, which has openings to allow the escape of the air and gases which are not retained in solution in the fume arrester.

The pipe 8 is carried into the central portion of the fume arrester and has a downwardly projecting end portion 12. The 65 fume arrester is charged with an acidulous solution, and the water line is indicated in dotted lines in the drawings.

Extending through the fume arrester is a shaft 13 carrying a pulley 14 at its upper 70 end, whereby said shaft may be rotated. Said shaft carries a wheel or radially projecting arms 15 near its lower end, which serves as a means to cause a circulation of the solution in the fume arrester, and thus 75 aids in drawing the fumes into the solution by the suction produced by the revolving of the wheel or arms.

An electrolytic cell 16 having the side portions 17 and the top portion 18, is connected by means of a pipe 19 with the fume arrester. A second pipe 20 located at a point above the pipe 19, also connects the cell with the fume arrester. The cell is provided with an acidulous solution. The pipes 80 19 and 20 will provide means whereby the solution in the fume arrester and the cell will be caused to circulate back and forth from one to the other, thus carrying the chlorids held in solution to the electrolytic 85 cell.

The electrolytic cell may be of any desired type, and as herein shown, is provided with a central porous carbon partition 21, which permits the solution to pass from one 95 side thereof to the other, but prevents the disintegrated carbon from corrupting the copper cathodes.

The chlorids in the solution will be disintegrated, the chlorin gas being liberated in 100 the usual manner at the carbon anode, while the metal collects at the copper cathode.

A pipe 22 leads from the electrolytic cell and connects with the pipe 7, so that the chlorin gas may be returned to the furnace 105 and re-used in the volatilization of the ores. If desired, a chlorin gas storage tank might be conveniently interposed between the pipes 22 and 7, and serve as a means for storing the chlorin gas until it is desired to be used. 110

While I have shown and described a particular form of fume arrester and electro-

lytic cell, it should be clearly understood that any other form of fume arrester may be used, and that any desired form of electrolytic cell may be used, the essential features being that the fumes containing the chlorids as they pass from the furnace will be caught in solution where the chlorids may be separated, and the chlorin gas liberated by the electrolytic action.

10 My improved process, therefore, which is preferably carried out by the apparatus above described, consists in treating the crushed ore with chlorin gas in a heated chamber, so that the ores are volatilized; 15 then passing the fumes out from the furnace through a fume arrester, where the chlorids are caught in solution; the separating of the chlorin gas from the chlorids by electrolytic action, and the passing of the 20 chlorin gas back to the furnace, where it may be re-used in the volatilization action in the furnace.

Any other form of apparatus may be used, if desired, in carrying out my process.

25 Having thus described my invention, what I claim as new and desire to secure by Letters Patent, is:—

1. The process of volatilizing the metals out of ores, consisting in treating the pul- 30 verized ore, either roasted or unroasted, in a hot chamber with chlorin gas, collecting

from said ore the fumes containing the chlorids of the metals, passing said fumes into an aqueous acid solution, separating the chlorin gas from the metals by electrolysis 35 in the solution, and again passing the reclaimed chlorin gas through the ore in the inclosed heating chamber, whereby said chlorin gas is re-used in the volatilization of the ores. 40

2. The process of volatilizing the metals out of ores, consisting in heating a closed chamber containing the ore and treating the ore in hot condition with chlorin gas, collecting from said ore the fumes containing 45 the chlorids of the metals, passing said fumes into an aqueous acid solution, separating the chlorin gas from the metals in the solution, and again passing the reclaimed chlorin gas through the ore in the inclosed heating 50 chamber, whereby said chlorin gas is re-used in the volatilization of the ores, and also serves as a carrier for conveying the metals from the ores to the solution, where said metals may be recovered. 55

In testimony whereof I affix my signature, in presence of two witnesses.

SELDEN IRWIN CLAWSON.

Witnesses:

W. H. THOMAS,  
HENRY THOMAS.